



US009244410B1

(12) **United States Patent**  
**Wu et al.**

(10) **Patent No.:** **US 9,244,410 B1**  
(45) **Date of Patent:** **Jan. 26, 2016**

(54) **FUSER MEMBER**

(71) Applicant: **Xerox Corporation**, Norwalk, CT (US)

(72) Inventors: **Jin Wu**, Pittsford, NY (US); **Matthew M. Kelly**, West Henrietta, NY (US); **Jonathan H. Herko**, Walworth, NY (US); **Lin Ma**, Pittsford, NY (US)

(73) Assignee: **Xerox Corporation**, Norwalk, CT (US)

(\*) Notice: Subject to any disclaimer, the term of this patent is extended or adjusted under 35 U.S.C. 154(b) by 0 days.

(21) Appl. No.: **14/623,791**

(22) Filed: **Feb. 17, 2015**

(51) **Int. Cl.**  
**G03G 15/20** (2006.01)

(52) **U.S. Cl.**  
CPC ..... **G03G 15/206** (2013.01)

(58) **Field of Classification Search**

None

See application file for complete search history.

(56) **References Cited**

U.S. PATENT DOCUMENTS

3,883,452 A \* 5/1975 Scheuerlein ..... C08J 9/26  
51/298  
3,917,761 A \* 11/1975 Scheuerlein ..... C08J 9/26  
264/126  
4,026,833 A \* 5/1977 D'Alelio ..... C08G 18/6438  
521/157  
4,026,871 A \* 5/1977 D'Alelio ..... C08G 18/6438  
525/422

4,058,505 A \* 11/1977 D'Alelio ..... C08G 18/6438  
525/354  
4,060,515 A \* 11/1977 D'Alelio ..... C08G 18/6438  
525/354  
4,197,397 A \* 4/1980 D'Alelio ..... C08G 73/1014  
528/125  
4,537,947 A \* 8/1985 D'Alelio ..... C08G 18/6438  
428/458  
8,753,735 B2 \* 6/2014 Gilmartin ..... C09D 5/24  
399/115  
2008/0038657 A1 \* 2/2008 Yamazaki ..... G03G 9/107  
430/120.4  
2008/0050138 A1 \* 2/2008 Yamazaki ..... G03G 15/235  
399/69  
2012/0213553 A1 \* 8/2012 Hoshio ..... G03G 15/0233  
399/176  
2012/0301818 A1 \* 11/2012 Gilmartin ..... G03G 15/0233  
430/66  
2012/0315060 A1 \* 12/2012 Sugiyama ..... G03G 15/2039  
399/69  
2013/0004205 A1 \* 1/2013 Gilmartin ..... G03G 15/0233  
399/176  
2015/0234329 A1 \* 8/2015 Hase ..... G03G 15/2039  
399/69

\* cited by examiner

Primary Examiner — David Gray

Assistant Examiner — Sevan A Aydin

(74) Attorney, Agent, or Firm — Hoffman Warnick LLC

(57) **ABSTRACT**

The present teachings provide a fuser member. The fuser member includes a substrate layer. The substrate layer includes a paraformaldehyde modified polyimide. An intermediate layer is disposed on the substrate layer. A release layer is disposed on the intermediate layer. A method of manufacturing the paraformaldehyde modified polyimide is disclosed.

**20 Claims, 5 Drawing Sheets**





FIG. 1



FIG. 2



FIG. 3



FIG. 4



FIG. 5

**1**  
**FUSER MEMBER**

BACKGROUND

1. Field of Use

This disclosure is generally directed to fuser members useful in electrophotographic imaging apparatuses, including digital, image on image, and the like. In addition, the fuser member described herein can also be used in a transfix apparatus in a solid ink jet printing machine.

2. Background

Polymers have many desirable properties for engineering systems including low mass density, chemical stability, and high strength-to-mass ratio. Polymeric materials typically have a low thermal conductivity near room temperature; in fact, foams of amorphous polymers are widely used for thermal insulation. In situations where heat transfer is critical, polymeric materials are at a disadvantage.

In the electrophotographic printing process, a toner image can be fixed or fused upon a support (e.g., a paper sheet) using a fuser member. Conductive fillers and fibers have been incorporated into polymeric materials to enhance conductivity of fuser members. However, incorporation of conductive fillers or fibers into polymeric material can decrease the Young's modulus of polymeric material. Incorporation of conductive fillers or fibers requires an additional processing step. It would be desirable to have a fuser belt having higher thermal conductivity, high thermal diffusivity and a high Young's modulus.

SUMMARY

According to an embodiment, a fuser member is provided. The fuser member includes a substrate layer of paraformaldehyde modified polyimide.

According to another embodiment, there is provided a fuser member. The fuser member includes a substrate layer of a paraformaldehyde modified polyimide. The fuser member includes an intermediate layer disposed on the substrate layer, the intermediate layer including a material selected from the group consisting of silicone and fluoroelastomer. A release layer is disposed on the intermediate layer, the release layer includes a fluoropolymer.

According to another embodiment there is provided a method of manufacturing a substrate layer for use in an electrophotographic machine. The method includes reacting a polyamic acid with a paraformaldehyde at a temperature of about 50° C. for about 30 minutes to form a polyamic acid network. The polyamic acid network onto a substrate and cured at a temperature of from about 200° C. to about 370° C. for a time of from about 30 minutes to about 150 minutes to form a paraformaldehyde cross-linked polyimide substrate layer.

BRIEF DESCRIPTION OF THE DRAWINGS

The accompanying drawings, which are incorporated in and constitute a part of this specification, illustrate several embodiments of the present teachings and together with the description, serve to explain the principles of the present teachings.

FIG. 1 depicts an exemplary fuser member having a belt substrate in accordance with the present teachings.

FIG. 2 depicts an exemplary fusing configuration using the fuser member shown in FIG. 1 in accordance with the present teachings.

**2**

FIG. 3 depicts an exemplary fusing configuration using the fuser member shown in FIG. 1 in accordance with the present teachings.

FIG. 4 depicts a fuser configuration using a transfix apparatus.

FIG. 5 depicts reaction flowchart for forming paraformaldehyde modified polyimide.

It should be noted that some details of the FIGS. have been simplified and are drawn to facilitate understanding of the 10 embodiments rather than to maintain strict structural accuracy, detail, and scale.

DESCRIPTION OF THE EMBODIMENTS

15 Reference will now be made in detail to embodiments of the present teachings, examples of which are illustrated in the accompanying drawings. Wherever possible, the same reference numbers will be used throughout the drawings to refer to the same or like parts.

20 In the following description, reference is made to the accompanying drawings that form a part thereof, and in which is shown by way of illustration specific exemplary embodiments in which the present teachings may be practiced. These embodiments are described in sufficient detail to enable those skilled in the art to practice the present teachings and it is to be understood that other embodiments may be utilized and that changes may be made without departing from the scope of the present teachings. The following description is, therefore, merely illustrative.

25 Illustrations with respect to one or more implementations, alterations and/or modifications can be made to the illustrated examples without departing from the spirit and scope of the appended claims. In addition, while a particular feature may have been disclosed with respect to only one of several implementations, such feature may be combined with one or more other features of the other implementations as may be desired and advantageous for any given or particular function. Furthermore, to the extent that the terms "including", "includes", "having", "has", "with", or variants thereof are used in either 30 the detailed description and the claims, such terms are intended to be inclusive in a manner similar to the term "comprising." The term "at least one of" is used to mean one or more of the listed items can be selected.

35 Notwithstanding that the numerical ranges and parameters 45 setting forth the broad scope of embodiments are approximations, the numerical values set forth in the specific examples are reported as precisely as possible. Any numerical value, however, inherently contains certain errors necessarily resulting from the standard deviation found in their respective testing measurements. Moreover, all ranges disclosed herein are to be understood to encompass any and all sub-ranges 50 subsumed therein. For example, a range of "less than 10" can include any and all sub-ranges between (and including) the minimum value of zero and the maximum value of 10, that is, any and all sub-ranges having a minimum value of equal to or 55 greater than zero and a maximum value of equal to or less than 10, e.g., 1 to 5. In certain cases, the numerical values as stated for the parameter can take on negative values. In this case, the example value of range stated as "less than 10" can assume negative values, e.g. -1, -2, -3, -10, -20, -30, etc.

60 The fuser or fixing member can include a substrate having one or more functional intermediate layers formed thereon. The substrate described herein includes a belt. The one or more intermediate layers include cushioning layers and release layers. Such fuser member can be used as an oil-less 65 fusing member for high speed, high quality electrophotographic printing to ensure and maintain a good toner release

from the fused toner image on an image supporting material (e.g., a paper sheet), and further assist paper stripping.

In various embodiments, the fuser member can include, for example, a substrate, with one or more functional intermediate layers formed thereon. The substrate can be formed in various shapes, such as a belt, or a film, using suitable materials that are non-conductive or conductive depending on a specific configuration, for example, as shown in FIG. 1.

In FIG. 1, an exemplary embodiment of a fusing or fix member 200 can include a belt substrate 210 with one or more functional intermediate layers, e.g., 220 and an outer surface layer 230 formed thereon. The outer surface layer 230 is also referred to as a release layer. The belt substrate 210 is described further and is made of paraformaldehyde modified polyimide.

#### Intermediate Layer or Functional Layer

Examples of materials used for the functional intermediate layer 220 (also referred to as cushioning layer or intermediate layer) include fluorosilicones, silicone rubbers such as room temperature vulcanization (RTV) silicone rubbers, high temperature vulcanization (HTV) silicone rubbers, and low temperature vulcanization (LTV) silicone rubbers. These rubbers are known and readily available commercially, such as SILASTIC® 735 black RTV and SILASTIC® 732 RTV, both from Dow Corning; 106 RTV Silicone Rubber and 90 RTV Silicone Rubber, both from General Electric; and JCR6115CLEAR HTV and SE4705U HTV silicone rubbers from Dow Corning Toray Silicones. Other suitable silicone materials include siloxanes (such as polydimethylsiloxanes); fluorosilicones such as Silicone Rubber 552, available from Sampson Coatings, Richmond, Va.; liquid silicone rubbers such as vinyl crosslinked heat curable rubbers or silanol room temperature crosslinked materials; and the like. Another specific example is Dow Corning Sylgard 182. Commercially available LSR rubbers include Dow Corning Q3-6395, Q3-6396, SILASTIC® 590 LSR, SILASTIC® 591 LSR, SILASTIC® 595 LSR, SILASTIC® 596 LSR, and SILASTIC® 598 LSR from Dow Corning. The functional layers provide elasticity and can be mixed with inorganic particles, for example SiC or Al<sub>2</sub>O<sub>3</sub>, as required.

Other examples of the materials suitable for use as functional intermediate layer 220 also include fluoroelastomers. Fluoroelastomers are from the class of 1) copolymers of two of vinylidenefluoride, hexafluoropropylene, and tetrafluoroethylene; such as those known commercially as VITON A® 2) terpolymers of vinylidenefluoride, hexafluoropropylene, and tetrafluoroethylene those known commercially as VITON B®; and 3) tetrapolymers of vinylidenefluoride, hexafluoropropylene, tetrafluoroethylene, and cure site monomer those known commercially as VITON GH® or VITON GF®. These fluoroelastomers are known commercially under various designations such as those listed above, along with VITON E®, VITON E 60C®, VITON E430®, VITON 910®, and VITON ETP®. The VITON® designation is a Trademark of E.I. DuPont de Nemours, Inc. The cure site monomer can be 4-bromoperfluorobutene-1,1,1-dihydro-4-bromoperfluorobutene-1,3-bromoperfluoropropene-1,1,1-dihydro-3-bromoperfluoropropene-1, or any other suitable, known cure site monomer, such as those commercially available from DuPont. Other commercially available fluoropolymers include FLUOREL 2170®, FLUOREL 2174®, FLUOREL 2176®, FLUOREL 2177® and FLUOREL LVS 76®, FLUOREL® being a registered trademark of 3M Company. Additional commercially available materials include AFLASTM a poly(propylene-tetrafluoroethylene), and FLUOREL IIR® (LII900) a poly(propylene-tetrafluoroethylene-vinylidenefluoride), both also available from 3M Com-

pany, as well as the Tecnoflons identified as FOR-60KIR®, FOR-LHF®, NM® FOR-THF®, FOR-TFS®, TH®, NH®, P757®, TNS®, T439®, PL958®, BR9151® and TN505®, available from Ausimont.

5 The fluoroelastomers VITON GH® and VITON GF® have relatively low amounts of vinylidenefluoride. The VITON GF® and VITON GH® have about 35 weight percent of vinylidenefluoride, about 34 weight percent of hexafluoropropylene, and about 29 weight percent of tetrafluoroethylene, with about 2 weight percent cure site monomer.

10 The thickness of the intermediate layer 220 is from about 30 microns to about 1,000 microns, or from about 100 microns to about 800 microns, or from about 150 microns to about 500 microns.

#### 15 Release Layer

An example embodiment of a release layer 230 includes fluoropolymer particles. Fluoropolymer particles suitable for use in the formulation described herein include fluorine-containing polymers. These polymers include fluoropolymers comprising a monomeric repeat unit that is selected from the group consisting of vinylidene fluoride, hexafluoropropylene, tetrafluoroethylene, perfluoroalkylvinylether, and mixtures thereof. The fluoropolymers may include linear or 20 branched polymers, and cross-linked fluoroelastomers. Examples of fluoropolymer include polytetrafluoroethylene (PTFE); perfluoroalkoxy polymer resin (PFA); copolymer of tetrafluoroethylene (TFE) and hexafluoropropylene (HFP); copolymers of hexafluoropropylene (HFP) and vinylidene 25 fluoride (VDF or VF2); terpolymers of tetrafluoroethylene (TFE), vinylidene fluoride (VDF), and hexafluoropropylene (HFP); and tetrapolymers of tetrafluoroethylene (TFE), vinylidene fluoride (VF2), and hexafluoropropylene (HFP), and mixtures thereof. The fluoropolymer particles provide 30 chemical and thermal stability and have a low surface energy. The fluoropolymer particles have a melting or curing temperature of from about 255° C. to about 360° C. or from about 280° C. to about 330° C. These particles are melted or cured 35 to form the release layer.

40 For the fuser member 200, the thickness of the outer surface layer or release layer 230 can be from about 10 microns to about 100 microns, or from about 20 microns to about 80 microns, or from about 40 microns to about 60 microns.

#### Adhesive Layer(s)

45 Optionally, any known and available suitable adhesive layer, also referred to as a primer layer, may be positioned between the release layer 230, the intermediate layer 220 and the substrate 210. Examples of suitable adhesives include silanes such as amino silanes (such as, for example, HV 50 Primer 10 from Dow Corning), titanates, zirconates, aluminates, and the like, and mixtures thereof. In an embodiment, an adhesive in from about 0.001 percent to about 10 percent solution can be wiped on the substrate. The adhesive layer can be coated on the substrate, or on the outer layer, to a thickness 55 of from about 2 nanometers to about 2,000 nanometers, or from about 2 nanometers to about 500 nanometers. The adhesive can be coated by any suitable known technique, including spray coating or wiping.

FIGS. 2 and 3 depict an exemplary fusing configuration for 60 the fusing process in accordance with the present teachings. It should be readily apparent to one of ordinary skill in the art that the fusing configurations 300B and 400B depicted in FIGS. 2 and 3, respectively, represent generalized schematic illustrations and that other members/layers substrates/configurations can be added or existing members/layers substrates/configurations can be removed or modified. Although 65 an electrophotographic printer is described herein, the dis-

closed apparatus and method can be applied to other printing technologies. Examples include offset printing and inkjet and solid transfix machines.

FIG. 2 depicts the fusing configuration 300B using a fuser belt shown in FIG. 1 in accordance with the present teachings. The configuration 300B can include a fuser belt of FIG. 1 that forms a fuser nip with a pressure applying mechanism 335, such as a pressure belt, for an image supporting material 315. In various embodiments, the pressure applying mechanism 335 can be used in combination with a heat lamp (not shown) to provide both the pressure and heat for the fusing process of the toner particles on the image supporting material 315. In addition, the configuration 300B can include one or more external heat rolls 350 along with, e.g., a cleaning web 360, as shown in FIG. 2.

FIG. 3 depicts the fusing configuration 400B using a fuser belt shown in FIG. 1 in accordance with the present teachings. The configuration 400B can include a fuser belt (i.e., 200 of FIG. 1) that forms a fuser nip with a pressure applying mechanism 435, such as a pressure belt in FIG. 3, for a media substrate 415. In various embodiments, the pressure applying mechanism 435 can be used in a combination with a heat lamp to provide both the pressure and heat for the fusing process of the toner particles on the media substrate 415. In addition, the configuration 400B can include a mechanical system 445 to move the fuser belt 200 and thus fusing the toner particles and forming images on the media substrate 415. The mechanical system 445 can include one or more rolls 445a-c, which can also be used as heat rolls when needed.

FIG. 4 demonstrates a view of an embodiment of a transfix member 7 which may be in the form of a belt, sheet, film, or like form. The transfix member 7 is constructed similarly to the fuser belt described above. The developed image 12 positioned on intermediate transfer member 1, is brought into contact with and transferred to transfix member 7 via rollers 4 and 8. Roller 4 and/or roller 8 may or may not have heat associated therewith. Transfix member 7 proceeds in the direction of arrow 13. The developed image is transferred and fused to a copy substrate 9 as copy substrate 9 is advanced between rollers 10 and 11. Rollers 10 and/or 11 may or may not have heat associated therewith.

#### Substrate Layer

The substrate layer 210 disclosed herein is a composition of paraformaldehyde modified polyimide.

The paraformaldehyde modified polyimide is derived from corresponding polyamic acids such as a polyamic acid of pyromellitic dianhydride/4,4'-oxydianiline, a polyamic acid of pyromellitic dianhydride/phenylenediamine, a polyamic acid of biphenyl tetracarboxylic dianhydride/4,4'-oxydianiline, a polyamic acid of biphenyl tetracarboxylic dianhydride/phenylenediamine, a polyamic acid of benzophenone tetracarboxylic dianhydride/4,4'-oxydianiline, a polyamic acid of benzophenone tetracarboxylic dianhydride/4,4'-oxydianiline/phenylenediamine, and the like, and mixtures thereof.

Commercially available examples of polyamic acids of pyromellitic dianhydride/4,4'-oxydianiline selected include PYRE-ML® RC-5019 (about 15 to 16 weight percent in N-ethyl-2-pyrrolidone, NMP), RC-5057 (about 14.5 to 15.5 weight percent in NMP/aromatic hydrocarbon, 80/20), and RC-5083 (about 18 to 19 weight percent in NMP/DMAc, 15/85), all available from Industrial Summit technology Corporation, and Parlin, N.J.; DURIMIDE® 100, commercially available from FUJIFILM Electronic Materials U.S.A., Incorporated.

Polyamic acids of biphenyl tetracarboxylic anhydride/phenylenediamine examples include U-VARNISH® A, and S

(about 20 weight percent in NMP), both available from UBE America Inc., New York, N.Y., BPDA resin (about 16.8 weight percent in NMP), available from Kaneka Corporation, TX, PI-2610 (about 10.5 weight percent in NMP), and PI-2611 (about 13.5 weight percent in NMP), both available from HD MicroSystems, Parlin, N.J.

Examples of polyamic acids of benzophenone tetracarboxylic dianhydride/4,4'-oxydianiline include RP46 and RP50 (about 18 weight percent in NMP), both available from Unitech Corp., Hampton, Va.

Polyamic acids of benzophenone tetracarboxylic dianhydride/4,4'-oxydianiline/phenylenediamine examples are PI-2525 (about 25 weight percent in NMP), PI-2574 (about 25 weight percent in NMP), PI-2555 (about 19 weight percent in NMP/aromatic hydrocarbon=80/20), and PI-2556 (about 15 weight percent in NMP/aromatic hydrocarbon/propylene glycol methyl ether=70/15/15), all available from HD MicroSystems, Parlin, N.J.

More specifically, polyamic acid or esters of polyamic acid examples that can be selected for the formation of a polyimide are prepared by the reaction of a dianhydride and a diamine. Suitable dianhydrides selected include aromatic dianhydrides and aromatic tetracarboxylic acid dianhydrides such as, for example, 9,9-bis(trifluoromethyl)xanthene-2,3,6,7-tetracarboxylic acid dianhydride, 2,2-bis(3,4-dicarboxyphenyl)hexafluoropropane dianhydride, 2,2-bis((3,4-dicarboxyphenoxy)phenyl)hexafluoropropane dianhydride, 4,4'-bis(3,4-dicarboxy-2,5,6-trifluorophenoxy)octafluorobiphenyl dianhydride, 3,3',4,4'-tetracarboxybiphenyl dianhydride, 3,3',4,4'-tetracarboxybenzophenone dianhydride, di-(4-(3,4-dicarboxyphenoxy)phenyl)ether dianhydride, di-(4-(3,4-dicarboxyphenoxy)phenyl) sulfide dianhydride, di-(3,4-dicarboxyphenyl)methane dianhydride, di-(3,4-dicarboxyphenyl)ether dianhydride, 1,2,4,5-tetracarboxybenzene dianhydride, 1,2,4-tricarboxybenzene dianhydride, butanetetracarboxylic dianhydride, cyclopantanetracarboxylic dianhydride, pyromellitic dianhydride, 1,2,3,4-benzenetetracarboxylic dianhydride, 2,3,6,7-naphthalenetetracarboxylic dianhydride, 1,4,5,8-naphthalenetetracarboxylic dianhydride, 1,2,5,6-naphthalenetetracarboxylic dianhydride, 3,4,9,10-perylene tetra carboxylic dianhydride, 2,3,6,7-anthracene tetracarboxylic dianhydride, 1,2,7,8-phenanthrenetetracarboxylic dianhydride, 3,3',4,4'-biphenyltetracarboxylic dianhydride, 2,2',3,3'-biphenyltetracarboxylic dianhydride, 3,3',4,4'-benzophenonetetracarboxylic dianhydride, 2,2',3,3'-benzophenonetetracarboxylic dianhydride, 2,2-bis(3,4-dicarboxyphenyl)propane dianhydride, 2,2-bis(2,3-dicarboxyphenyl)propane dianhydride, bis(3,4-dicarboxyphenyl)ether dianhydride, bis(2,3-dicarboxyphenyl)ether dianhydride, bis(3,4-dicarboxyphenyl)sulfide dianhydride, bis(2,3-dicarboxyphenyl)sulfide dianhydride, 2,2-bis(3,4-dicarboxyphenyl)-1,1,3,3-hexafluoropropane dianhydride, 2,2-bis(3,4-dicarboxyphenyl)-1,1,3,3-hexachloropropane dianhydride, 1,1-bis(2,3-dicarboxyphenyl)ethane dianhydride, 1,1-bis(3,4-dicarboxyphenyl)ethane dianhydride, bis(2,3-dicarboxyphenyl)methane dianhydride, bis(3,4-dicarboxyphenyl)methane dianhydride, 4,4'-(p-phenylenedioxy)diphtalic dianhydride, 4,4'-(m-phenylenedioxy)diphtalic dianhydride, 4,4'-diphenylsulfidedioxobis(4-phthalic acid) dianhydride, 4,4'-diphenylsulfonedioxobis(4-phthalic acid) dianhydride, methylenebis(4-phenyleneoxy-4-phthalic acid) dianhydride, ethylidenebis(4-phenyleneoxy-4-phthalic acid) dianhydride, isopropylidenebis(4-phenyleneoxy-4-phthalic acid)dianhydride, hexafluoroisopropylidenebis(4-phenyleneoxy-4-phthalic acid)dianhydride, and the like.

60

65

Exemplary diamines suitable for use in the preparation of the polyamic acids include 4,4'-bis-(m-aminophenoxy)-biphenyl, 4,4'-bis-(m-aminophenoxy)-diphenyl sulfide, 4,4'-bis-(m-aminophenoxy)-diphenyl sulfone, 4,4'-bis-(p-aminophenoxy)-benzophenone, 4,4'-bis-(p-aminophenoxy)-diphenyl sulfide, 4,4'-bis-(p-aminophenoxy)-diphenyl sulfone, 4,4'-diamino-azobenzene, 4,4'-diaminobiphenyl, 4,4'-diaminodiphenylsulfone, 4,4'-diamino-p-terphenyl, 1,3-bis-(gamma-aminopropyl)-tetramethyl-disiloxane, 1,6-diaminohexane, 4,4'-diaminodiphenylmethane, 3,3'-diamino-diphenylmethane, 1,3-diaminobenzene, 4,4'-diaminodiphenyl ether, 2,4'-diaminodiphenylether, 3,3'-diaminodiphenylether, 3,4'-diaminodiphenylether, 1,4-diaminobenzene, 4,4'-diamino-2,2',3,3',5,5',6,6'-octafluorobiphenyl, 4,4'-diamino-2,2',3,3',5,5',6,6'-octafluorodiphenyl ether, bis[4-(3-aminophenoxy)-phenyl]sulfide, bis[4-(3-aminophenoxy)phenyl]sulfone, bis[4-(3-aminophenoxy)phenyl]ketone, 4,4'-bis(3-aminophenoxy)biphenyl, 2,2-bis[4-(3-aminophenoxy)phenyl]-propane, 2,2-bis[4-(3-aminophenoxy)phenyl]-1,1,1,3,3,3-hexafluoropropane, 4,4'-diaminodiphenyl sulfide, 4,4'-diaminodiphenyl ether, 4,4'-diaminodiphenyl sulfone, 4,4'-diaminodiphenylmethane, 1,1-di(p-aminophenyl)ethane, 2,2-di(p-aminophenyl)propane, and 2,2-di(p-aminophenyl)-1,1,1,3,3,3-hexafluoropropane, and the like, and mixtures thereof.

The dianhydrides and diamines are, for example, selected in a weight ratio of from about 20:80 to about 80:20, a weight ratio of from about 60/40 to about 40/60 and about a 50:50 weight ratio.

Various amounts of polyamic acid can be selected for the substrate, such as for example, from about 60 weight percent to about 99.5 weight percent, from about 70 weight percent to about 99 weight percent, or from about 90 weight percent to about 98 weight percent based on the total weight of the substrate.

Various amounts of paraformaldehyde can be selected for the substrate such as for example, from about 0.5 weight percent to about 40 weight percent, from about 1 weight percent to about 10 weight percent, or from about 2 weight percent to about 10 weight percent based on the total weight of the substrate.

The method of making the paraformaldehyde modified polyimide substrate is illustrated in FIG. 5. The polyamic acid is reacted with paraformaldehyde at a temperature of about 0° C. to about 50° C. for about 10 minutes to about 180 minutes. When the reaction is completed, it is theorized that a hemiaminal network of polyamic acid is formed as shown in FIG. 5. The hemiaminal network of polyamic acid is coated onto a substrate and cured with heat although other polyamic networks could be formed. The curing of the hemiaminal network of polyamic acid results in a hexahydrotriazine cross-linked polyimide. The hexahydrotriazine cross-linked polyimide is removed from the substrate after cooling is used as a fuser member. However, not wanting to be bound by theory, other cross-linked polyimides with the paraformaldehyde could be formed by the disclosed process.

The substrate can optionally contain a polysiloxane copolymer to enhance or smooth the coating. The concentration of the polysiloxane copolymer is from about 0.01 weight percent to about 1.0 weight percent based on the total weight of the substrate. The optional polysiloxane copolymer includes a polyester modified polydimethylsiloxane, commercially available from BYK Chemical with the trade name of BYK® 310 (about 25 weight percent in xylene) and 370 (about 25 weight percent in xylene/alkylbenzenes/cyclohexanone/monophenylglycol=75/11/7/7); a polyether modified polydimethylsiloxane, commercially available from BYK

Chemical with the trade name of BYK® 330 (about 51 weight percent in methoxypropylacetate) and 344 (about 52.3 weight percent in xylene/isobutanol=80/20), BYK®-SILCLEAN 3710 and 3720 (about 25 weight percent in methoxypropylacetate); a polyacrylate modified polydimethylsiloxane, commercially available from BYK Chemical with the trade name of BYK®-SILCLEAN 3700 (about 25 weight percent in methoxypropylacetate); or a polyester polyether modified polydimethylsiloxane, commercially available from BYK Chemical with the trade name of BYK® 375 (about 25 weight percent in Di-propylene glycol monomethyl ether).

Additives and additional conductive or non-conductive fillers may be present in the above-described substrate layer, intermediate layer or release layer. In various embodiments, other filler materials or additives including, for example, inorganic particles, can be used. Fillers used herein include carbon blacks, aluminum nitride, boron nitride, aluminum oxide, graphite, graphene, copper flake, nano diamond, carbon nanotube, metal oxide, doped metal oxide, metal flake, and mixtures thereof. In various embodiments, other additives known to one of ordinary skill in the art can also be included to form the disclosed composite materials.

The network of polyamic acid composition is flow coated onto a substrate and cured. The curing of the hemiaminal network of polyamic acid composition is at a temperature of from about 200° C. to about 370° C., or from about 300° C. to about 340° C., for a time of from about 30 minutes to about 150 minutes, or from about 60 minutes to about 120 minutes. The curing can be done in stages with the composition under tension in the final stage.

## EXAMPLES

35 Experimentally, a polyamic acid of biphenyl tetracarboxylic dianhydride/p-benzenediamine (BPDA resin from Kaneka, about 16.6 weight percent in NMP, dark brown) was mixed with paraformaldehyde and additional NMP solvent with a mechanical mixer at the weight ratio of 95/5 at 50° C. for 30 minutes, and a bright orange solution was formed. After coating the solution and subsequent curing at 170° C. for 30 minutes and 320° C. for 120 minutes, a paraformaldehyde modified polyimide belt was obtained for fuser belt application. A controlled polyimide belt without any paraformaldehyde modification was similarly prepared.

The resulting polyimide composite belt was tested and possessed significantly higher thermal diffusivity and thermal conductivity than the control polyimide belt. The thermal diffusivity and thermal conductivity was obtained using the LFA 447 Nanoflash instrument. The results are summarized in Table 1.

TABLE 1

|                                                    | Paraformaldehyde<br>Polyimide | modified polyimide |
|----------------------------------------------------|-------------------------------|--------------------|
| Thermal diffusivity (mm <sup>2</sup> /s) at 25° C. | 0.1985                        | 0.3617             |
| Thermal diffusivity (mm <sup>2</sup> /s) at 20° C. | 0.1445                        | 0.227              |
| Thermal conductivity (W/(m° K.)) at 25° C.         | 0.2963                        | 0.5374             |
| Thermal conductivity (W/(m° K.)) at 20° C.         | 0.3498                        | 0.5732             |

In summary, disclosed herein is a paraformaldehyde modified polyimide fuser belt having higher thermal diffusivity and thermal conductivity without the addition of inorganic fillers. This eliminates the dispersion process step during manufacture where an inorganic filler is incorporated polyimide fuser belt.

It will be appreciated that variants of the above-disclosed and other features and functions or alternatives thereof may be combined into other different systems or applications. Various presently unforeseen or unanticipated alternatives, modifications, variations, or improvements therein may be subsequently made by those skilled in the art, which are also encompassed by the following claims.

What is claimed is:

1. A fuser member comprising:

a substrate layer comprising a paraformaldehyde modified polyimide, wherein paraformaldehyde is from about 0.5 weight percent to about 40 weight percent of the substrate layer and polyimide is from about 60 weight percent to about 99.5 weight percent of the substrate layer.

2. The fuser member of claim 1, further comprising an intermediate layer disposed on the substrate layer; and a release layer disposed on the intermediate layer.

3. The fuser member of claim 2, wherein the intermediate layer comprises silicone.

4. The fuser member of claim 2, wherein the release layer comprises a fluoropolymer.

5. The fuser member of claim 1, wherein the substrate layer further comprises a polysiloxane polymer.

6. The fuser member of claim 5, wherein the polysiloxane polymer is selected from the group consisting of: a polyester modified polydimethylsiloxane, a polyether modified polydimethylsiloxane, a polyacrylate modified polydimethylsiloxane, and a polyester polyether modified polydimethylsiloxane.

7. The fuser member of claim 5, wherein the polysiloxane polymer comprises from about 0.01 weight percent to about 1.0 weight percent of the substrate layer.

8. The fuser member of claim 1, wherein the substrate layer further comprises at least one filler.

9. The fuser member of claim 8, wherein the at least one filler is selected from the group consisting of: aluminum nitride, boron nitride, aluminum oxide, graphite, graphene, copper flake, nano diamond, carbon black, carbon nanotube, metal oxides, doped metal oxide, metal flake, poly(p-phenylene benzobisoxazole) fiber and aramid fiber.

10. A fuser member comprising:

a substrate layer comprising a paraformaldehyde modified polyimide;

an intermediate layer disposed on the substrate layer comprising a material selected from the group consisting of: silicone and fluoroelastomer; and

a release layer disposed on the intermediate layer, the release layer comprising a fluoropolymer.

11. The fuser member of claim 10, wherein the substrate layer further comprises a polysiloxane polymer.

12. The fuser member of claim 11, wherein the polysiloxane polymer is selected from the group consisting of: a polyester modified polydimethylsiloxane, a polyether modified polydimethylsiloxane, a polyacrylate modified polydimethylsiloxane, and a polyester polyether modified polydimethylsiloxane.

13. The fuser member of claim 11, wherein the polysiloxane polymer comprises from about 0.01 weight percent to about 1.0 weight percent of the substrate layer.

14. The fuser member of claim 10, wherein the substrate layer further comprises at least one filler.

15. The fuser member of claim 14, wherein the at least one filler is selected from the group consisting of: aluminum nitride, boron nitride, aluminum oxide, graphite, graphene, copper flake, nano diamond, carbon black, carbon nanotube, metal oxides, doped metal oxide, metal flake, poly(p-phenylene benzobisoxazole) fiber and aramid fiber.

16. A method of manufacturing a substrate layer for use in an electrophotographic machine, the method comprising:

reacting a polyamic acid with a paraformaldehyde at a temperature of about 0° C. to about 60° C. for about 10 minutes to about 180 minutes to form a polyamic acid network;

coating the polyamic acid network onto a substrate; and curing the polyamic network at a temperature of from about 200° C. to about 370° C. for a time of from about 30 minutes to about 150 minutes to form a paraformaldehyde cross-linked polyimide substrate layer.

17. The method of claim 16, wherein the polyamic acid network comprises a hemiaminal network of polyamic acid.

18. The method of claim 16, wherein the paraformaldehyde cross-linked polyimide substrate layer comprises hexahydridotriazine cross-linked polyimide.

19. The method of claim 16, wherein the polyamic acid is selected from the group consisting of a polyamic acid of pyromellitic dianhydride/4,4'-oxydianiline, a polyamic acid of pyromellitic dianhydride/phenylenediamine, a polyamic acid of biphenyl tetracarboxylic dianhydride/4,4'-oxydianiline, a polyamic acid of biphenyl tetracarboxylic dianhydride/phenylenediamine, a polyamic acid of benzophenone tetracarboxylic dianhydride/4,4'-oxydianiline, a polyamic acid of benzophenone tetracarboxylic dianhydride/4,4'-oxydianiline/phenylenediamine, and mixtures thereof.

20. The method of claim 16, wherein paraformaldehyde is from about 0.5 weight percent to about 40 weight percent of the paraformaldehyde cross-linked polyimide substrate layer and polyimide is from about 60 weight percent to about 99.5 weight percent of the substrate layer the paraformaldehyde cross-linked polyimide substrate layer.

\* \* \* \* \*